

1

3,016,143

**FLOTATION OF GRANULAR ORES**  
**Joseph E. Trachta and Carlos O. Rodriguez, Carlsbad,**  
**N. Mex., assignors to International Minerals & Chemical**  
**Corporation, a corporation of New York**  
**No Drawing. Filed Dec. 19, 1958, Ser. No. 781,462**  
**10 Claims. (Cl. 209—166)**

The present invention relates to the separation of minerals in granular form. More particularly, it relates to the separation of a granular mixture of minerals by selective flotation of a component thereof. In one embodiment, it relates to the flotation of sylvite from granular sylvinitite of the type occurring in the Carlsbad, New Mexico, area.

The separation of mixed minerals into their component species by selective flotation is now a well-established procedure in the minerals beneficiation art. In all cases, it is necessary for the mineral to be crushed or otherwise reduced in size sufficiently to liberate the mineral components from one another, and it is generally necessary for the mineral to be crushed to a particle size not greater than about 30 mesh in order to carry out a successful flotation. Larger particles are much more difficult to separate by flotation, since it is correspondingly more difficult for the air bubbles to become attached thereto in a quantity sufficiently great to lift the particles.

For many purposes, however, it is most undesirable to reduce the mineral to powdery form. In the manufacture and utilization of fertilizers, for example, which commonly include phosphate rock and sylvite or other potash mineral, the use of such materials in finely divided form gives rise to caking and dusting problems, so that granular materials are distinctly preferred, and the demand therefor has greatly expanded within recent years. A need has therefore existed for a method of beneficiating such materials in granular form, so that they are directly available to the market without any necessity for separating them first in powdered form and then re-converting them into granular form.

Methods have already been devised which achieve flotation of granular materials to some extent. Such methods generally subject an aqueous slurry of the desired mineral to aeration in the presence of a selective reagent such as an amine or a fatty acid, a frothing agent such as an aliphatic alcohol of intermediate molecular weight, and a non-saponifiable oil such as crude petroleum, fuel oil, or kerosene. These methods are reasonably effective, but leave much to be desired in terms of product recovery and product quality. The present invention is an improvement in such a process, whereby the product recovery is increased and the product quality is improved.

One object of the present invention is to separate the components of a granular mixture of substances.

Another object is to improve the flotation of granular mixtures.

Another object is to separate granular ores into their component substances.

Another object is to separate granular sylvite in improved yield and quality from coarse granular sylvinitite.

Another object is to improve the quality of flotation-grade granular sylvite.

Other objects of the invention will be apparent from the present description and claims.

2

The present invention achieves a more selective and more complete flotation of a desired ore component from a granular mixture thereof by adding to the flotation mixture a viscous petroleum oil having certain critical characteristics and specifications. In order to improve the product grade and recovery, the oil should have a pour point of 50° F. to 120° F., a viscosity above about 100 SSU at 130° F., and below 300 SSU, preferably above about 150 SSU, and should be largely a high-boiling material, having a distillation temperature above about 500° F. at the 10% distillation level. If it is further desired to avoid darkening of the product during the final drying operation, the oil should meet additional specifications. Specifically, it should be largely distillable, leaving a residue of not more than about 15% and preferably not more than about 5%. It should have a distillation end point at ordinary pressure below about 1000° F., preferably below about 900° F. It should have a Conradson carbon below about 5% and preferably below about 1%. It should desirably, but not necessarily, be comprised of 35% to 100% paraffinic hydrocarbons. It can contain up to 65% aromatic and naphthenic hydrocarbons without adversely affecting flotation.

The foregoing specifications are summarized and amplified in the following table.

Distillation range (ASTM D-447):

|                                       |                  |
|---------------------------------------|------------------|
| IBP, °F.—                             |                  |
| 10%—                                  | Over 500.        |
| 30 90%—                               | Over 600.        |
| EP—                                   | Below 1000.      |
| Distillation recovery, percent—       | Over 85.         |
| Viscosity, SSU, 130° F.—              | Over 100 to 300. |
| Conradson carbon, percent—            | Below 5.         |
| 35 Unsulfonatable materials, percent— | Over 35.         |
| Analysis, percent—                    |                  |
| Aromatics plus naphthenes—            | 0—65.            |
| Paraffins—                            | 35—100.          |
| Pour point, °F.—                      | 50° to 120°.     |

From the foregoing specifications it will be apparent that the oils conventionally employed in mineral flotation are incapable of producing the improved results of the present invention. Crude oils of various types are too wide in boiling range, and are often too high in asphaltic content for optimum flotation performance. Gasoline and kerosine fractions produce negligible flotation and are actually harmful. Diesel oil fractions produce float concentrations of high analysis, but with very low recovery. Other light fuel oils behave somewhat similarly.

Suitable oil fractions for use in the present invention include the so-called "gas oils," lubricating oil stocks, and paraffin or wax distillates obtained in the distillation of crude oils and in the redistillation of cracked stocks and heavy distillates. All of these materials produce the improved results of the invention, so long as they meet the specifications noted above.

The oil is employed in a proportion between about 2 and about 5 pounds per ton of solids. Somewhat lower proportions may be employed if desired, but at a penalty with respect to product recovery; and somewhat higher proportions may be employed if desired, but generally with some degree of reduction in product grade.

In one embodiment of the invention, a sylvinitite ore is crushed to liberation of the sylvite constituent, sized to 65 around —10 +28 mesh, placed in brine (i.e., a saturated

aqueous solution of sylvinitic ore), deslimed, slurried to about 65% solids, reagentized with an aliphatic amine such as n-laurylamine in the form of its acetate salt, and subjected to a conventional froth flotation in the presence of methyl isobutyl carbinol as a frothing agent and in the presence of a viscous petroleum fraction as hereinabove described. The float concentrate, comprising largely sylvite, is withdrawn, dewatered, washed if desired, and dried. Excellent recoveries, around 80-90% or higher, are obtained, and the product has an analysis around 60% K<sub>2</sub>O.

The invention is applicable generally to the flotation of granular ore mixtures, and is employed in connection with conventional techniques for such purpose. The granular ore, preferably after being sized and deslimed, is made into a slurry with a suitable brine at a total solids level of about 65% by weight or higher, the maximum proportion being limited so as to obtain a fluid slurry. Into this mixture is incorporated a suitable reagent, the type of reagent being chosen according to the nature of the ore and the particular component which is desired to be floated. If, for example, sylvite is to be floated from sylvinitic ore or from sylvinitic-langbeinitic mixed ore, a cationic reagent is employed, such as n-laurylamine, n-octadecylamine, or other aliphatic amine, preferably in the form of the acetate, hydrochloride, or other water-soluble acid addition salt. The choice of a suitable flotation reagent in a given case is well known to the art, and does not form a novel part of the present invention.

It is also conventional to incorporate in the flotation mixture a suitable frothing agent, such as an aliphatic alcohol of intermediate molecular weight (around C<sub>4</sub>-C<sub>10</sub>), a preferred example being methyl isobutyl carbinol. Other frothing agents are described in the art.

A preferred type of oil for use in the present invention is a fractionator still bottoms obtained in the fractionation of a catalytic cracking unit product in refining crude oil from Eddy and Lea Counties, New Mexico, at the Malco Refinery, Artesia, New Mexico. In obtaining such a material, crude oil is first distilled at reduced pressure until an overhead vapor temperature of about 700° F. is attained. The overhead fraction obtained by vacuum distillation at about 700° F. is termed vacuum gas oil and is a suitable flotation reagent. This stock oil is fed to a catalytic cracking unit from which fractionator bottoms, a preferred flotation oil, is obtained.

The following table lists pertinent physical and chemical properties of a typical fractionator bottoms and a typical vacuum gas oil suitable for use in the present invention:

|                                       | Fractionator<br>Bottoms | Vacuum<br>Gas Oil |
|---------------------------------------|-------------------------|-------------------|
| Distillation range, ° F.:             |                         |                   |
| IBP Corrected to one atmosphere       | 265                     | 585               |
| 10% Corrected to one atmosphere       | 510                     | 675               |
| 50% Corrected to one atmosphere       | 715                     | 820               |
| 90% Corrected to one atmosphere (85%) | 875                     | 945               |
| EP Corrected to one atmosphere (85%)  | 875                     | 975               |
| Distillation recovery, percent        | 85                      | 97.5              |
| Viscosity, SSU:                       |                         |                   |
| 100° F.                               | 310                     | 300               |
| 130° F.                               | 153                     | 148               |
| 210° F.                               | 51                      | 52                |
| Pour point, ° F.                      | 80-90                   | 90-100            |
| Index of refraction                   | 1.543                   | 1.520             |
| API gravity                           | 18.5                    | 21.2              |
| Sp. gr. 60/60° F.                     | 0.9433                  | 0.9267            |
| Ash, percent                          | 0.0                     | 0.0               |
| Conradson carbon, percent             | 2.2                     | 0.3               |
| Sulfur, percent                       | 1.98                    | 0.80              |
| Unsulfonatable material, percent      | 60                      | 70                |
| Molecular weight                      | 302                     | 355               |
| Analysis:                             |                         |                   |
| Paraffins+naphthenes                  | 50.5                    | 56.0              |
| Aromatics                             | 49.5                    | 44.0              |

It is feasible in many cases to employ a blend of oils to improve one or more characteristics of the flotation product. It has been found, for example, that a blend of a light lube oil stock and a crude oil fractionator bottoms

in around 50:50 ratio by volume gives higher product recovery and grade than either component alone. For such a blend, it is advantageous to employ a distillate fraction with a fractionator bottoms fraction, the latter serving to maximize the viscosity, while the former reduces the proportion of color-forming bodies. Blends in various proportions may of course be employed, depending upon the color tolerance of the product and the desired product recovery.

The invention will be more readily understood from the following operating examples.

#### Example 1

A flotation-grade crude oil obtained from Lynch Station, Lea County, New Mexico, was fractionally distilled into the following five fractions:

|                  | Percent (by volume) |
|------------------|---------------------|
| Gasoline         | 10                  |
| Kerosine         | 10                  |
| Diesel oil       | 10                  |
| Light lube stock | 24                  |
| Still bottoms    | 46                  |

Flotation tests were carried out on each fraction, employing a thoroughly deslimed -8 +28 mesh sylvinitic ore fraction containing 17.4% K<sub>2</sub>O in a saturated brine at 65% solids content. The slurry was reagentized with T.D. amine (Armeen TD, n-octadecylamine) at 0.85 pound per ton. Methyl isobutyl carbinol was used as a frothing agent in the proportion of 1.1 lbs./ton. The oil was used in the proportion of 10.3 lbs./ton. The tests were carried out according to conventional procedure, using a Fagergren laboratory test machine adapted for granular flotation. The results were as follows:

| Oil                   | K <sub>2</sub> O Content            |                         | K <sub>2</sub> O Recovery | Remarks                                                      |
|-----------------------|-------------------------------------|-------------------------|---------------------------|--------------------------------------------------------------|
|                       | Concen-<br>trate<br>Percent<br>60.9 | Tails<br>Percent<br>3.1 |                           |                                                              |
| Crude<br>Gasoline     |                                     |                         | 86.6                      | Control Test.<br>Poor Flotation.                             |
| Kerosine              | 61.1                                | 9.3                     | Not measurable.<br>do.    | Do.                                                          |
| Diesel                | 61.1                                | 9.3                     | 54.9                      | Natural color<br>concentrate.<br>do.                         |
| Lube<br>Bottoms       | 62.2                                | 5.4                     | 75.2                      | Dark color<br>concentrate.<br>do.                            |
| 50:50<br>Lube+Bottoms | 58.9                                | 2.5                     | 89.4                      | Dark color<br>concentrate.<br>Improved color<br>concentrate. |
| 50:50<br>Lube+Bottoms | 60.6                                | 2.0                     | 91.5                      |                                                              |

#### Example 2

A plant-scale test was carried out to compare a highly paraffinic fractionator bottoms material produced at the Malco Oil Co. refinery at Artesia, New Mexico, with a mixed base crude oil conventionally employed for granular flotation of sylvite from sylvinitic. The flotation feed was 35 tons per hour of deslimed -8 +28 mesh sylvinitic ore having a grade of 15.6% K<sub>2</sub>O, slurried in saturated brine to 65% solids for conditioning, reagentized with TD-Armeen octadecylamine hydrochloride, and employing methyl isobutyl carbinol as the frothing agent.

During a 4-day period employing crude oil, an indicated recovery of 83.3% was obtained with an amine consumption of 0.99 lb./ton, an alcohol usage of .048 lb./ton and an oil usage of 4.5 lbs./ton.

During the ensuing four days, employing the fractionator bottoms, an indicated recovery of 86.3% was obtained with an amine usage of 0.84 lb./ton, an alcohol usage of .030 lb./ton, and an oil usage of 3.7 lbs./ton.

During the four days after usage of the crude oil had been resumed, the indicated recovery was again 83.3% with an amine usage of 0.95 lb./ton, an alcohol usage of .048 lb./ton and an oil usage of 4.5 lbs./ton.

During the test period employing fractionator bottoms, the tailings contained an average of only 1.8% K<sub>2</sub>O, while the unleached concentrate contained 56.9% K<sub>2</sub>O.

## Example 3

Tests were similarly carried out to compare the fractionator bottoms with a vacuum gas oil from the same refinery. The results were as follows:

|                                    | Test No. 1 |                       | Test No. 2 |                       |
|------------------------------------|------------|-----------------------|------------|-----------------------|
|                                    | Vacuum Oil | Frac-tionator Bottoms | Vacuum Oil | Frac-tionator Bottoms |
| Oil usage, lbs./ton                | 3.7        | 4.6                   | 4.3        | 3.4                   |
| Amine usage, lbs./ton              | .092       | .085                  | .092       | .089                  |
| K <sub>2</sub> O content, percent: |            |                       |            |                       |
| Feed                               | 16.7       | 15.7                  | 13.8       | 12.9                  |
| Concentrate                        | 59.2       | 59.0                  | 58.8       | 57.3                  |
| Tails                              | 3.3        | 2.5                   | 1.9        | 2.5                   |
| Indicated recovery, percent        | 85.0       | 87.8                  | 88.4       | 84.3                  |

The foregoing examples refer to a number of starting materials and a number of specific instances of the class of oils to which the present invention relates. It is to be understood that such matters are illustrative only, and are not intended by way of limitation. Numerous other examples of the invention and alternative ways and aspects in which it can be applied will readily be apparent from the foregoing description to those skilled in the art.

The invention is generally applicable to the separation of the components of coarse granular ores such as sylvinite, langbeinite, carnallite, polyhalite, mixed sylvinite-langbeinite ore, phosphate pebble ore, and other ores which can be separated by flotation at particle sizes larger than those normally used for froth flotation. The foregoing description refers principally to the treatment of sylvinite ores, but it will be recognized that the invention is equally applicable wherever a product of large particle size is desired, for example, a Florida phosphate ore of -3 +35 mesh size. The present process requires a feed material of a particle size not greater than about 3 mesh, and sufficiently small to effect economical liberation of the desired material from the gangue. It also requires that the materials be separable by flotation means. Except in these respects, the invention is not limited as to starting material.

The following claims particularly point out and distinctly claim the subject matter of the invention:

1. In a process for separating the components of a granular potash ore wherein one component of said ore is selectively floated in the presence of a selective reagent for said component, a frothing agent, and a petroleum oil fraction, the improvement which comprises employing as said fraction a petroleum fraction having a viscosity at 130° F. greater than about 100 SSU, more than 35% unsulfonatable materials, and a distillation range with a 10% point above about 500° F.

2. A process as in claim 1 wherein said petroleum oil fraction has a viscosity at 130° F. between about 100 SSU and about 300 SSU.

3. A process as in claim 1 wherein said petroleum oil

fraction has a Conradson carbon below about 5% and a distillation range having an end point below about 1000° F.

4. A process as in claim 1 wherein said petroleum oil fraction has a Conradson carbon below about 1% and a distillation range having an end point below about 900° F.
5. A process as in claim 1 wherein said petroleum oil fraction is a gas oil fraction.
6. A process as in claim 1 wherein said petroleum oil fraction is a lube oil fraction.
7. A process as in claim 1 wherein said petroleum oil fraction is a wax oil distillate fraction.
8. In a process for separating the components of a granular potash ore having a particle size between about 3 and about 35 mesh wherein one component of said ore is selectively floated in the presence of a selective reagent for said component, a frothing agent, and a petroleum oil, the improvement which comprises employing as said oil a crude oil distillation residue having a viscosity at 130° F. greater than about 100 SSU, more than 35% unsulfonatable materials, and a distillation range having a 10% point above about 500° F. and an end point below about 1000° F.
9. In a process for separating the components of a granular potash ore having a particle size between about 3 and about 35 mesh wherein one component of said ore is selectively floated in the presence of a selective reagent for said component, a frothing agent, and a petroleum oil, the improvement which comprises employing as said oil a blend of a crude oil distillation residue and a lube oil fraction, said blend having a viscosity at 130° F. greater than about 100 SSU, more than 35% unsulfonatable materials, and a distillation range having a 10% point about 500° F. and an end point below about 1000° F.
10. In a process for selectively floating sylvite from granular sylvite ore, which process comprises sizing sylvite to the range of about -3 +35 mesh, desliming and then slurrying with a saturated sylvite brine in a proportion to produce a fluent slurry containing above about 65% solids, incorporating therein a cationic reagent, a frothing agent, and a petroleum oil, and subjecting said slurry to aeration to selectively remove the sylvite as a froth concentrate, the improvement which comprises employing as said petroleum oil a petroleum fraction having a viscosity at 130° F. above about 100 SSU, more than 35% unsulfonatable materials, a distillation range having a 10% point above about 500° F. and an end point below about 1000° F., and a Conradson carbon below about 5%, whereby the grade and recovery of said sylvite are substantially improved, and whereby discoloration of the product is largely avoided.

## References Cited in the file of this patent

## UNITED STATES PATENTS

- 1,830,908 Luckenback Nov. 10, 1931  
 2,420,476 Greene et al. May 13, 1947  
 2,839,192 Monson June 17, 1958